

J. L. HERMAN.

PROCESS OF COATING AND TREATING MATERIALS HAVING AN IRON BASE.

APPLICATION FILED FEB. 10, 1922.

1,430,648.

Patented Oct. 3, 1922.



By

Inventor

Joseph L. Herman

Frank A. Poole

Attorney

## UNITED STATES PATENT OFFICE.

JOSEPH L. HERMAN, OF PEORIA, ILLINOIS.

## PROCESS OF COATING AND TREATING MATERIALS HAVING AN IRON BASE.

Application filed February 10, 1922. Serial No. 535,660.

*To all whom it may concern:*

Be it known that I, JOSEPH L. HERMAN, a citizen of the United States, a resident of Peoria, in the county of Peoria and State of Illinois, have invented new and useful Improvements in Processes of Coating and Treating Materials Having an Iron Base, of which the following is a specification.

This invention has reference to a process 10 of coating and treating materials having an iron base and particularly the coating and treatment of wire used in the fence industry and for telephone and other purposes.

The principal object of the invention is 15 to subject the coated material to a heat-treatment during the continuous process of coating such material and preferably immediately upon the material leaving the molten bath in which the material is immersed or through which the material is 20 immersed or through which the material is moving. Such heat-treatment has for its object an improved coating which will be more resistant to atmospheric rusting and corroding conditions than is ordinary galvanized wire, and which further will permit 25 a heavier coated wire to be used in wire fabricating machines without causing the coating to crack or flake off, as is the case with heavily coated galvanized wire coated 30 by ordinary processes.

The invention has for a further object to 35 apply a heavier coating on the wire with a shorter immersion in molten zinc than is the case with ordinary galvanized wire carrying heavier coating and the elimination of the usual wiping mechanism, or the necessity for wiping.

A further object of the invention is to permit the use of higher speeds for galvanizing 40 wire than can be done under the ordinary galvanizing process and at the same time causing a heavier coating to be formed on the wire.

Galvanized wire which is to be used for 45 fabricating purposes and more particularly that which is to be used in the manufacture of woven wire fencing must have a relatively heavy coating of spelter in order to be able to withstand atmospheric corroding conditions, and before my invention was 50 developed this was not possible except at a much increased cost of production.

The universal practice for testing the relative value of spelter on galvanized wire is 55 by the so-called Preece or copper sulfate

test. There are other tests, however, which are used for quantitatively determining the amount of spelter on galvanized wire, such as stripping the coating in caustic soda solution; in a suitable hydrochloric acid solution; in a solution of hydrochloric acid and antimony chloride, and in a lead acetate solution. The copper sulfate test, although not strictly quantitative, is comparative when used under known conditions of temperature and strength, and being a quick test, and one which can be performed by any one after a little experience, has come to be the routine testing medium for galvanized wire 60 coatings.

At the present time there are only two (2) methods in use whereby these necessary heavy zinc (spelter) coatings may be obtained by the hot process of galvanizing. The first method is to pass the wire, as it 70 emerges from the galvanizing bath, through finely divided charcoal. By such a process a smooth, thick coating may be obtained. This method is used for making telephone wire. It has serious drawbacks, however, 75 from an economic standpoint, because the wire must travel at a very slow speed, a very high grade zinc must be used, and, furthermore, the coated wire cannot be subjected to the action of wire-fence fabricating machines without having considerable of the zinc coating crack or flake off the iron base. The second method is to cause the wire to travel at relatively slow speeds, through a 80 bath of molten spelter, the speed depending on the gauge of wire, the thickness of coating desired and the length of the molten spelter bath, and then wiping the wire by passing it between suitable wipes. In other words, a wire will have a heavier galvanized 85 coating, as measured by the copper sulfate test, the longer it remains in the molten spelter. This latter process, too, has its economic drawbacks, because of the slow speeds required, the long spelter pans necessary and consequently the lessening of the tonnage passing through a galvanizing unit in a given time.

By the use of my invention I am not only 90 permitted to use high speeds for galvanizing wire but I also obviate the necessity of using wipes or other smoothing mediums, the latter being heretofore considered indispensable by all wire galvanizers. The 95 reason for this is due to the operation of my 100

70

75

80

85

90

95

100

105

110

heat-treater which not only heat-treats per se, but also evens up the coating as though it had been passed between wipers. Another advantage in eliminating the wipers 5 is that a heavier coat is permitted to remain on the wire, which in ordinary practice is removed by the wipers, as the wire is passed therethrough. It will therefore be apparent to those skilled in the art that the higher 10 speeds can be used because it is not necessary for the wire to remain immersed in the molten bath for as long a period of time as is necessary in the ordinary galvanizing practice.

15 In the accompanying drawing there is illustrated diagrammatically the usual or ordinary continuous galvanizing or coating apparatus including the "annealing furnace," "acid" bath, "flux" bath, "coating" or 20 galvanizing bath, and my "heat-treater" associated therewith, by means of which my process may be carried out.

25 My process consists in treating wire as is usual in the ordinary continuous galvanizing of wire, and I have discovered that if instead of carrying spelter at the temperatures ordinarily used in wire galvanizing practice, i. e., 840° F. to 880° F., it is carried at, say, 950° to 1000° Fahrenheit, and 30 that after leaving the spelter passing the wire through heat of, say, 1200° Fahrenheit, I have a superior galvanized product. For example, if a No. 12 gauge wire (American steel wire gauge) is passed through molten 35 spelter carried at a temperature of approximately 1000° Fahrenheit for approximately two seconds and then through heat of approximately 1200° Fahrenheit for approximately seven seconds, and with or without 40 wiping after leaving the heat treatment, a wire is coated which will stand approximately four one minute immersions in copper sulfate; whereas a similar wire traveling through the spelter at the same time and 45 speed as the treated wire and wiped after leaving the spelter, and not passing through the heat-treatment, will stand, as a general rule, not over one minute immersion in copper sulfate. If the latter wire (which I 50 call the control wire) is not passed through a wipe of some kind after it leaves the spelter, then, although I obtain a wire which will stand more than one copper sulfate immersion test, it is very rough, an uncom- 55 mercial, unsalable product, and cannot be successfully used in fence fabricating machines.

60 What I have described for No. 12 gauge wire is also true for other gauges of wire, some of the larger gauges such as No. 9 standing oftentimes many more than four copper sulfate immersion tests. I do not, of course, limit myself to the speeds and temperatures above given because I have found 65 that I may vary the speeds by controlling

the temperatures; for example, if I want the wire to travel at a high speed, then I use higher temperatures, and vice versa.

In an application of my process, I subject a No. 12 gauge wire to a bath of molten spelter held at a temperature approximately 70 950° Fahrenheit for approximately one and one-half seconds. Immediately upon the wire emerging from the spelter it enters a tube heated at approximately 1250° Fahrenheit 75 and remains in this tube subjected to this heat for approximately seven seconds. The wire then passes to a reel upon which it is coiled. I find that the heat-treatment to which the wire is exposed not only permits 80 a uniform coating to be carried on the wire but the coating is also heavier than is the case if I pass the wire through the usual wipers as it leaves the coating bath and not subjecting the same to the heat-treatment. 85 "Heat-treatment" as employed by me has reference to such treatment as will produce a physical or chemical change in the material undergoing treatment. Furthermore, the fact that I do not wipe the coating as it 90 leaves the spelter bath allows a heavier coating to remain upon the wire, this coating being both uneven and brittle if stopped at this point. When, however, the coated wire is subjected to the action of my heat-treatment it not only causes this heavy coat to 95 distribute itself evenly around the wire, but it also eliminates the brittleness referred to above. I find that there is an apparent bonding action taking place possibly due to 100 some kind of an alloying action caused by the heat, and although I have determined the improvement in the coating over that of an ordinary galvanized coating by several hundred tests I am not yet fully aware as 105 to the exact physical and chemical changes which take place.

The example above given is only one of very many examples which could be cited developed out of actual practice and for 110 that reason I do not wish to limit myself to temperatures, speeds or gauges of wire as specified above. I have used various gauges of wire from No. 6 to No. 17 and I have used spelter temperatures as high as 1275° 115 Fahrenheit and I have carried my heater as high as 1450° Fahrenheit. These are not at all limiting gauges or temperatures but are merely cited to show the multitude of combinations possible.

I have also found that when I carry my heat-treater toward the higher range of temperature, such as I have quoted above that I may pass my coated wire therethrough at a higher rate of speed than is the case when 125 my heat-treater is close to the lower end of the range specified. This is particularly true because the larger sizes of wire are usually caused to travel at a speed relatively slower than the smaller sizes of wire. 130

For example if I am galvanizing a No. 17 gauge wire I may use a speed of one hundred feet per minute. The temperature of the spelter bath may be 1200° Fahrenheit 5 and the temperature of the heat-treater may only be 900° Fahrenheit. On the other hand, the same size wire may be traveling at the rate of one hundred fifty feet per minute and the spelter bath temperature may be 10 900° Fahrenheit; whereas, the heat-treater might be carried at 1275° Fahrenheit. The foregoing example illustrates in what manner I may carry the heat-treater at a relatively high temperature as compared to the 15 coating bath, and vice versa, and it also indicates that by varying the speed of the wire I may also vary the temperatures of either the heat-treater, the spelter bath, or both because it is a known fact and old in the art 20 that the longer the wire is immersed in the spelter within reasonable limits the heavier will be the coating, even though the wire be wiped. I have shown previously, however, that before my process economic use could 25 not be made of the latter fact to equal that produced by my process. It is therefore obvious to those skilled in the art that modifications of the foregoing may be made without departing from the spirit and scope of 30 the invention.

Wire galvanized by my process has an exceptionally smooth coating even without the use of wipes. This gives me another advantage, in that I eliminate the production of "reachers" which, with the ordinary galvanizing practice are always produced and as such are valueless except as scrap. Furthermore, it is not necessary for me to use excessively long spelter pans, as I have 40 eliminated the necessity for long immersion of the wire in molten spelter.

I am aware that attempts have been made to treat metal coated metallic materials by subjecting the same to a heat treatment 45 after coating. Such processes, however, have been intermittent and not continuous and required a heat-treatment at intervals of time ranging from not less than ten minutes to at least six hours and more, and at 50 temperatures ranging from approximately 400 to about 600 degrees Fahrenheit. Such processes as I have just referred to are economically impossible to use for the continuous process of galvanizing wire, for reasons 55 which are so obvious to those skilled in the art that comment is unnecessary.

What I claim is:

1. The process of treating metal coated materials having an iron base which consists 60 in heat-treating the coated materials at a

relatively low temperature as compared with the temperature at which such materials are coated, and continuously moving such materials through the heat.

2. The process of treating metal coated materials having an iron base which consists in heat-treating the coated materials at a relatively high temperature as compared with the temperature at which such materials are coated, and continuously moving 70 such materials through the heat.

3. The process of treating metal coated materials having an iron base which consists in heat-treating the coated materials and continuously moving such materials 75 through the heat, the temperature of which is dependent upon the speed at which the material is moved.

4. The process of treating metal coated materials having an iron base which consists in heat-treating the coated materials and continuously moving such materials through the heat, the speed at which the materials are moved being dependent upon the temperature to which the materials are 85 heated.

5. The process of galvanizing wire, which consists in continuously moving the wire and during such movement subjecting the same, first—to a molten bath of spelter and 90 upon leaving the bath subjecting the coated wire to a heat-treatment.

6. The process of galvanizing wire, which consists in continuously moving the wire and during such movement subjecting the 95 same, first—to a molten bath of spelter; second—removing the wire from the bath without wiping and finally subjecting the coated wire to a heat-treatment.

7. The process of galvanizing wire, which consists in continuously moving the wire and during such movement subjecting the same, first—to a molten bath of spelter; second—removing the wire from the bath without wiping and finally subjecting the coated 105 wire to a heat-treatment and removing the coated wire therefrom without wiping.

8. The process of treating galvanized wire which consists in heat-treating the coated wire and continuously moving such wire 110 through the heat, the temperature of the heat and the speed at which the wire is moved being dependent on the gauge of the wire and thickness of the galvanized coating.

In witness whereof I have hereunto affixed my hand this 3rd day of February, 1922.

JOSEPH L. HERMAN.